

[54] LUBRICANT COMPOSITIONS  
CONTAINING TERPOLYMERS[75] Inventor: Rudolf J. A. Eckert, Amsterdam,  
Netherlands

[73] Assignee: Shell Oil Company, New York, N.Y.

[22] Filed: Jan. 25, 1971

[21] Appl. No.: 109,674

## Related U.S. Application Data

[63] Continuation of Ser. No. 776,778, Nov. 18, 1968,  
abandoned.

## [30] Foreign Application Priority Data

Nov. 27, 1967 United Kingdom ..... 53761

[52] U.S. Cl..... 252/49.8, 260/80.71

[51] Int. Cl. .... C10m 1/46, C10m 1/28

[58] Field of Search ..... 252/49.8; 260/80 PS, 80.71

## [56]

## References Cited

## UNITED STATES PATENTS

|           |        |                        |            |
|-----------|--------|------------------------|------------|
| 3,208,943 | 2/1965 | Kirby.....             | 252/49.8   |
| 2,737,496 | 3/1956 | Catlin.....            | 252/51.5   |
| 3,030,303 | 4/1962 | Ryan .....             | 252/51.5 X |
| 3,192,158 | 6/1965 | Bergstrom et al. ..... | 252/51.5 X |
| 3,423,367 | 1/1969 | Merijan et al. .....   | 252/51.5 X |

Primary Examiner—Daniel E. Wyman

Assistant Examiner—W. Cannon

Attorney—Harold L. Denkler

## [57]

## ABSTRACT

Lubricating compositions containing a terpolymer of ethylene, with an alkyl ester of an unsaturated carboxylic acid, and with an olefinically unsaturated compound containing either a phosphorus atom or a heterocyclic nitrogen atom exhibit good thermal stability, viscosity index, and dispersant properties.

4 Claims, No Drawings

## LUBRICANT COMPOSITIONS CONTAINING TERPOLYMERS

This application is a continuation of application Ser. No. 776,778 filed Nov. 18, 1968, now abandoned.

This invention relates to novel lubricant compositions containing as additives polymeric compounds which, in addition to dispersant properties, also have viscosity-improving characteristics. The invention further relates to novel polymeric compounds which are suitable for use as lubricant additives.

A number of polymeric compounds have been proposed which are capable of imparting dispersant properties and improving the viscosity index of lubricating oils. A disadvantage of most of these compounds is that they possess a low thermal stability. If the lubricant in which they have been incorporated is exposed to high temperature, they are decomposed, as a result of which their favorable action is significantly reduced or disappears entirely. Therefore, when lubricants are exposed to high temperature, such as in combustion engines, it is desirable that the additives incorporated in the lubricants should possess a sufficiently high thermal stability, so that their favorable activity is retained.

A class of polymeric compounds has now been found which impart dispersant properties to a lubricating oil, improve the viscosity characteristics of the lubricating oil and possess, moreover, a very high thermal stability.

The invention therefore relates to novel lubricant compositions comprising one or more lubricants and terpolymers of one or more olefinically unsaturated hydrocarbons with one or more alkyl esters of unsaturated carboxylic acids and with one or more olefinically unsaturated compounds containing either a phosphorus atom or a heterocyclic nitrogen atom. The invention relates in particular to lubricant compositions comprising polymers selected from a class of terpolymers of olefinically unsaturated C<sub>2-8</sub> hydrocarbons with alkyl esters of unsaturated C<sub>3-5</sub> carboxylic acids, in which the alkyl groups contain eight-20 carbon atoms and with C<sub>2-10</sub> olefinically unsaturated compounds containing a phosphorus atom or a heterocyclic nitrogen atom.

Terpolymers which have been found to be particularly advantageous as additives to mineral lubricating oils include the following novel compounds:

1. ethylene/lauryl methacrylate/stearyl methacrylate/diethyl iso-propylidene phosphonate terpolymer,
2. ethylene/diisooctyl itaconate/diethyl isopropylidene phosphonate terpolymer,
3. ethylene/lauryl methacrylate/stearyl methacrylate/N-vinyl-2-pyrrolidone terpolymer,
4. ethylene/diisooctyl itaconate/N-vinyl-2-pyrrolidone terpolymer,
5. ethylene/lauryl methacrylate/stearyl methacrylate/2-vinyl pyridine terpolymer.

Base oils suitable for the preparation of the lubricant compositions according to the invention are mineral lubricating oils of varying viscosity, synthetic lubricating oils or lubricating oils containing fatty oils. The present lubricant additives may also be incorporated in lubricating greases. The invention is of special importance for improving the quality of mineral lubricating oils or mixtures thereof. The polymeric compounds can be added to the lubricant as such or in the form of a

concentrate obtained, for example, by mixing the polymeric compounds with a small quantity of oil. The concentration of the present polymers in the lubricant can vary between wide limits. In general, the desired dispersant action and improvement of the viscometric properties is obtained when the quantity added is from 0.1 to 10%w and in particular when this quantity is from 0.5 to 5%w of the lubricating composition.

In addition to the present polymers, the lubricant compositions according to the invention can also contain other additives, such as antioxidants, anti-corrosive agents, anti-foaming agents, agents to improve the lubricating action, and other substances which are usually added to lubricants.

The polymeric compounds incorporated into the lubricating compositions of the present invention are terpolymers of one or more olefinically unsaturated C<sub>2-8</sub> hydrocarbons, with one or more C<sub>8-20</sub> alkyl esters of C<sub>3-5</sub> carboxylic acids and with one or more C<sub>2-10</sub> olefinically unsaturated compounds containing either a phosphorus or a heterocyclic nitrogen atom.

The olefinically unsaturated hydrocarbons suitable for use as monomers in the preparation of the present terpolymers can be either aliphatic or aromatic hydrocarbons. Examples of suitable olefinically unsaturated aliphatic hydrocarbons are monoolefins, such as ethylene, propylene, butene and pentene, and diolefins, such as butadiene, isoprene and dimethylbutadiene. An example of a suitable olefinically unsaturated aromatic hydrocarbon is styrene. Preference is given to terpolymers which are prepared from ethylene. Terpolymers which have been prepared from diolefins may be used in lubricant compositions as such or may be hydrogenated thereby saturating at least part of the olefinically unsaturated bonds.

The alkyl esters of unsaturated carboxylic acids suitable for use as monomers in the preparation of the present terpolymers can be either alkyl esters of unsaturated monobasic carboxylic acids or alkyl esters of unsaturated polybasic carboxylic acids. Examples of suitable alkyl esters of unsaturated monobasic carboxylic acids are methyl methacrylate, isobutyl acrylate, lauryl methacrylate and stearyl methacrylate. Some examples of suitable alkyl esters of unsaturated polybasic carboxylic acids are diethyl maleate, diethyl fumarate and diisooctyl itaconate. Preference is given to polymers prepared from alkyl esters of monobasic or dibasic carboxylic acids, the alkyl groups of which contain eight-20 carbon atoms. Particularly advantageous alkyl ester monomers are diisooctyl itaconate or mixtures of lauryl and stearyl methacrylates.

Examples of olefinically unsaturated compounds containing either a phosphorus atom or a heterocyclic nitrogen atom are vinyl phosphonic acid and alkyl and aryl esters thereof, isopropylidene phosphonic acid and alkyl and aryl esters thereof, such as diethyl isopropylidene phosphonate, N-vinyl-2-pyrrolidone, 2-vinyl pyridine, 4-vinyl pyridine, N-vinyl carbazole, N-vinyl-2-oxazolidone, N-vinyl succinimide, 4-vinyl pyrimidine and 2-vinyl quinoline. Preference is given to polymers prepared from diethyl isopropylidene phosphonate or N-vinyl-2-pyrrolidone, or 2-vinyl pyridine.

Employing the aforementioned preferred monomers, the following novel compounds have been found to be particularly advantageous in improving the viscosity,

dispersant properties and thermal stability of lubricating oils:

1. ethylene/lauryl methacrylate/stearyl methacrylate/diethyl isopropylidene phosphonate terpolymer
2. ethylene/diisooctyl itaconate/diethyl isopropylidene phosphonate terpolymer
3. ethylene/lauryl methacrylate/stearyl methacrylate/N-vinyl-2-pyrrolidone terpolymer
4. ethylene/diisooctyl itaconate/N-vinyl-2-pyrrolidone terpolymer
5. ethylene/lauryl methacrylate/stearyl methacrylate/2-vinyl pyridine terpolymer.

The copolymerization of olefinically unsaturated hydrocarbons, alkyl esters of unsaturated carboxylic acids and olefinically unsaturated compounds containing either a phosphorus atom or a heterocyclic nitrogen atom is preferably conducted in solution in the presence of a free radical initiator, such as an azo compound or a peroxide.

The ratio in which the monomers are incorporated into a growing polymer molecule depends on the reactivity of the monomers involved. If there are differences in reactivity, the molar ratio of the monomers in the mixture to be polymerized will be subject to considerable changes as the copolymerization proceeds, since the more reactive monomer is incorporated more rapidly. As a result, the composition of the copolymer also changes continually. As a general rule it may be said that, if in the copolymerization of monomers which differ strongly in reactivity no special measures are taken, the products obtained are of an extremely heterogeneous composition. Such a case arises in the copolymerization of olefinically unsaturated hydrocarbons, alkyl esters of unsaturated carboxylic acids and olefinically unsaturated compounds containing either a phosphorus atom or a heterocyclic nitrogen atom, since three types of monomers are involved which differ in reactivity. In the copolymerization of these monomers it has been found that despite the very different reactivity it is possible to prepare copolymers with a constant average composition, if care is taken that the ratio between the concentrations of the monomers in the mixture remains constant during the copolymerization. This can be accomplished by adding additional quantities of the more reactive monomers or a mixture of monomers rich in reactive monomers to the mixture being polymerized. This method is known as programmed copolymerization. It is also possible to stop the polymerization when the concentrations of the monomers in the mixture to be polymerized are substantially the same. This is called copolymerization to low conversion.

The copolymerization of the present monomers may be conducted either batchwise or continuously. Continuous polymerization may take place in a tubular reactor or by continuously adding the reaction com-

ponents in the ratio in which they are consumed during the reaction. The composition is kept homogeneous by intensive stirring while simultaneously discharging part of the reaction mixture.

The molecular weight of the terpolymers can vary between wide limits. The invention relates in particular to lubricant compositions containing terpolymers with a molecular weight ( $M_n$ ) between 5,000 and 150,000, more specifically to lubricant compositions containing copolymers with a molecular weight between 10,000 and 80,000.

The ratio of the molar concentrations of the monomers can also vary within wide limits. The molar ratio of the monomers in the terpolymer is generally from 11 to 300 moles of olefinically unsaturated hydrocarbon to 10 moles of alkyl esters of unsaturated carboxylic acids to 1 to 15 moles of the olefinically unsaturated phosphorus or nitrogen containing monomer.

The invention will now be further described with the aid of the following examples.

#### EXAMPLE I

Four terpolymers of ethylene, lauryl methacrylate, stearyl methacrylate and N-vinyl-2-pyrrolidone, two terpolymers of ethylene, diisooctyl itaconate and N-vinyl-2-pyrrolidone, four terpolymers of ethylene, lauryl methacrylate, stearyl methacrylate and 2-vinyl pyridine, two terpolymers of ethylene, diisooctyl itaconate and diethyl isopropylidene phosphonate and three terpolymers of ethylene, lauryl methacrylate, stearyl methacrylate and diethyl isopropylidene phosphonate, were prepared using the procedure described below (polymers 1 to 15 incl.). Other compositions illustrative of the invention are terpolymers of styrene, diisooctyl itaconate and 2-vinyl pyridine; terpolymers of butadiene, diisooctyl itaconate and isopropylidene phosphonate, and terpolymers of dimethylbutadiene, stearyl and lauryl methacrylates, and N-vinyl-2-pyrrolidone.

A mixture of alkyl esters of unsaturated carboxylic acids, olefinically unsaturated compounds containing a phosphorus atom or a heterocyclic nitrogen atom, azodiisobutyronitrile and 400 g of benzene was passed into a 2-liter autoclave. After the air had been expelled from the autoclave with the aid of pure nitrogen, ethylene was introduced into the autoclave at room temperature under a pressure of up to 170 to 200 atm. The mixture was heated at 65°C for a certain period, during which the pressure increased to 400–500 atm. After the pressure had been released, the mixture was discharged and concentrated by partial evaporation of the solvent. The polymer was purified by precipitating three times in methanol. Finally the polymer was dissolved in benzene, the solution filtered and the polymer separated by freeze-drying.

Further data on the copolymerizations and the resulting terpolymers are given in Tables I and II.

TABLE I

| Polymer No.                                               | 1    | 2    | 3    | 4    | 5    | 6    | 7    | 8    | 9    | 10  | 11   | 12   | 13   | 14   | 15   |
|-----------------------------------------------------------|------|------|------|------|------|------|------|------|------|-----|------|------|------|------|------|
| Quantity of monomer in the mixture to be polymerized, g.: |      |      |      |      |      |      |      |      |      |     |      |      |      |      |      |
| Lauryl methacrylate                                       | 35.5 | 35.5 | 17.8 | 8.9  |      | 16.9 | 15.0 | 13.5 | 12.5 | 5.0 |      | 10.0 | 10.0 |      |      |
| Stearyl methacrylate                                      | 20.3 | 20.3 | 10.2 | 5.1  |      | 9.6  | 8.5  | 7.7  | 7.1  | 6.8 |      | 13.6 | 13.6 |      |      |
| Diisooctyl itaconate                                      |      |      |      |      | 35.4 | 17.7 |      |      |      |     |      | 14.2 |      | 28.3 |      |
| N-vinyl-2-pyrrolidone                                     | 36.0 | 48.0 | 36.0 | 36.0 | 36.0 | 36.0 |      |      |      |     |      |      |      |      |      |
| 2-vinyl pyridine                                          |      |      |      |      |      |      | 1.7  | 1.9  | 2.3  | 2.4 |      |      |      |      |      |
| Diethyl isopropylidene phosphonate                        |      |      |      |      |      |      |      |      |      |     | 10.0 | 10.0 | 20.0 | 30.0 | 20.0 |

TABLE I - Continued

| Polymer No.                                                            | 1      | 2      | 3      | 4      | 5      | 6      | 7      | 8     | 9      | 10     | 11     | 12     | 13     | 14     | 15     |
|------------------------------------------------------------------------|--------|--------|--------|--------|--------|--------|--------|-------|--------|--------|--------|--------|--------|--------|--------|
| Quantity of azodiisobutyronitrile in the mixture to be polymerized, g. | 0.2    | 0.2    | 0.15   | 0.12   | 0.15   | 0.12   | 0.12   | 0.18  | 0.18   | 0.18   | 0.15   | 0.15   | 0.2    | 0.2    | 0.2    |
| Duration of copolymerization, h.                                       | 3      | 2.5    | 3      | 3      | 3      | 3      | 3      | 3.5   | 3      | 4      | 4      | 3      | 3      | 3      | 3      |
| Yield of copolymer, g.                                                 | 21.7   | 26.7   | 8.0    | 1.4    | 21.4   | 13.3   | 2.3    | 2.6   | 3.1    | 2.1    | 7.6    | 9.5    | 8.1    | 11.9   | 17.0   |
| Average molecular weight of the terpolymers ( $M_n$ )                  | 44,500 | 34,500 | 28,000 | 24,100 | 18,500 | 18,500 | 16,006 | 8,250 | 16,290 | 15,900 | 32,500 | 21,800 | 28,500 | 36,000 | 12,800 |

TABLE II

| Polymer No. | Molar ratio of the monomers in terpolymer |                      |                      |                       |                  |                                    |          | Nitrogen content, wt. percent | Phosphorus content, wt. percent |
|-------------|-------------------------------------------|----------------------|----------------------|-----------------------|------------------|------------------------------------|----------|-------------------------------|---------------------------------|
|             | Lauryl methacrylate                       | Stearyl methacrylate | Diisooctyl itaconate | N-vinyl-2-pyrrolidone | 2-vinyl pyridine | Diethyl isopropylidene phosphonate | Ethylene |                               |                                 |
| 1           | 7                                         | 3                    |                      | 1.6                   |                  |                                    |          | 16                            | 0.66                            |
| 2           | 7                                         | 3                    |                      | 2.2                   |                  |                                    |          | 20                            | 0.85                            |
| 3           | 7                                         | 3                    |                      | 2.3                   |                  |                                    |          | 32.6                          | 0.80                            |
| 4           | 7                                         | 3                    |                      | 4.8                   |                  |                                    |          | 68                            | 1.3                             |
| 5           |                                           |                      | 10                   | 3.5                   |                  |                                    |          | 34.7                          | 1.0                             |
| 6           |                                           |                      | 10                   | 4.5                   |                  |                                    |          | 38.6                          | 1.23                            |
| 7           | 7                                         | 3                    |                      |                       | 3                |                                    |          | 14                            | 1.21                            |
| 8           | 7                                         | 3                    |                      |                       | 2.4              |                                    |          | 34                            | 0.86                            |
| 9           | 7                                         | 3                    |                      |                       | 3.3              |                                    |          | 36                            | 1.1                             |
| 10          | 7                                         | 3                    |                      |                       | 3.7              |                                    |          | 37                            | 1.22                            |
| 11          | 5                                         | 5                    |                      |                       |                  | 2.4                                |          |                               |                                 |
| 12          |                                           |                      | 10                   |                       |                  | 1.6                                |          | 78                            | 0.82                            |
| 13          | 5                                         | 5                    |                      |                       |                  | 1.8                                |          | 19                            | 1.48                            |
| 14          | 5                                         | 5                    |                      |                       |                  | 4.0                                |          | 49                            | 2.5                             |
| 15          |                                           |                      | 10                   |                       |                  | 2.2                                |          | 52                            | 1.24                            |

## EXAMPLE II

In order to assess their viscometric behavior, polymers 1-15 of Example I were dissolved in a concentration of 1.5%w in a paraffinic base oil. The results of the viscometric determinations are listed in Table III. 30

Table III

|                            | $V_k$ 100°F<br>cS | $V_k$ 210°F<br>cS | VI  | VT | 35 | 10  | 11  | 12  | 13  | 14  | 15  | 35    |
|----------------------------|-------------------|-------------------|-----|----|----|-----|-----|-----|-----|-----|-----|-------|
| Base oil                   | 57.77             | 7.36              | 96  | —  |    | 335 | 365 | 390 | 395 | 395 | 390 | 0.007 |
| Base oil + 1.5% polymer 1  | 79.69             | 9.97              | 113 | 93 |    | 355 | 370 | 395 | 395 | 395 | 395 | 0.007 |
| Base oil + 1.5% polymer 2  | 75.53             | 9.50              | 111 | 94 |    | 365 | 380 | 405 | 405 | 405 | 405 | 0.009 |
| Base oil + 1.5% polymer 3  | 76.27             | 9.55              | 111 | 92 |    | 355 | 370 | 405 | 405 | 405 | 405 | 0.012 |
| Base oil + 1.5% polymer 4  | 77.71             | 9.70              | 111 | 92 |    | 340 | 350 | 365 | 365 | 365 | 365 | 0.035 |
| Base oil + 1.5% polymer 5  | 66.44             | 8.39              | 104 | 92 |    | 360 | 370 | 395 | 395 | 395 | 395 | 0.035 |
| Base oil + 1.5% polymer 6  | 70.78             | 8.88              | 107 | 91 | 40 | 335 | 345 | 365 | 365 | 365 | 365 | 0.004 |
| Base oil + 1.5% polymer 7  | 68.56             | 8.64              | 106 | 92 |    | 345 | 355 | 385 | 385 | 385 | 385 | 0.004 |
| Base oil + 1.5% polymer 8  | 72.10             | 8.96              | 107 | 87 |    | 335 | 350 | 370 | 370 | 370 | 370 | 0.005 |
| Base oil + 1.5% polymer 9  | 71.51             | 8.86              | 106 | 85 |    | 340 | 355 | 390 | 390 | 390 | 390 | 0.020 |
| Base oil + 1.5% polymer 10 | 70.45             | 8.76              | 105 | 86 |    | 340 | 350 | 375 | 375 | 375 | 375 | 0.025 |
| Base oil + 1.5% polymer 11 | 84.90             | 10.43             | 112 | 88 |    | 340 | 350 | 365 | 365 | 365 | 365 | 0.025 |
| Base oil + 1.5% polymer 12 | 75.82             | 9.42              | 109 | 89 |    | 335 | 345 | 365 | 365 | 365 | 365 | 0.035 |
| Base oil + 1.5% polymer 13 | 78.86             | 9.78              | 111 | 90 | 45 | 335 | 345 | 365 | 365 | 365 | 365 | 0.035 |
| Base oil + 1.5% polymer 14 | 75.23             | 9.39              | 110 | 91 |    | 335 | 345 | 365 | 365 | 365 | 365 | 0.035 |
| Base oil + 1.5% polymer    | 66.55             | 8.39              | 104 | 91 |    | 335 | 345 | 365 | 365 | 365 | 365 | 0.004 |

The results shown in Table III indicate that the polymers of the present invention are very effective in improving the viscosity index of the paraffinic base oil.

## EXAMPLE III

The thermal stabilities of the polymers according to the invention are recorded in Table IV. They were determined in vacuum at a rate of heating of 3°C/min. The values  $T_{10}$ ,  $T_{20}$  and  $T_{50}$  represent the temperatures at which 10, 20 and 50 percent weight loss, respectively, of the polymer was attained.

To test the present polymers as dispersants they were subjected to a peptization test. In this test the lowest concentration of additive is determined that is capable of keeping 0.015%w of carbon in mineral oil in suspension for 15 minutes at 250°C. The results of these peptization tests are also listed in Table IV. These results show that all the polymers tested had a significant activity as dispersants. (Values of less than 0.05 reflect good dispersancy.)

Table IV

| Polymer | $T_{10}$ | $T_{20}$ | $T_{50}$ | Peptization Test, %w |
|---------|----------|----------|----------|----------------------|
| 1       | 355      | 365      | 390      | 0.007                |
| 2       | 355      | 370      | 395      | 0.007                |
| 3       | 365      | 380      | 405      | 0.009                |
| 4       | 355      | 370      | 405      | 0.012                |
| 5       | 340      | 350      | 365      | 0.035                |
| 6       | 360      | 370      | 395      | 0.035                |
| 7       | 335      | 345      | 365      | 0.004                |
| 8       | 345      | 355      | 365      | 0.004                |
| 9       | 345      | 360      | 385      | 0.004                |
| 10      | 335      | 350      | 370      | 0.004                |
| 11      | 340      | 355      | 390      | 0.005                |
| 12      | 330      | 340      | 380      | 0.020                |
| 13      | 340      | 350      | 375      | 0.025                |
| 14      | 340      | 350      | 365      | 0.025                |
| 15      | 335      | 345      | 365      | 0.035                |

The foregoing data clearly establish that the polymeric additives of the present invention impart good dispersant properties and improve the viscosity index of lubricating oils and also improve the thermal stability of the lubricant composition.

I claim as my invention:

1. A lubricating composition consisting essentially of a major amount of a mineral lubricating oil and from 0.1 to 10 percent by weight of an oil soluble terpolymer of (1) ethylene with (2) a  $C_{8-20}$  alkyl ester of a  $C_{3-5}$  unsaturated carboxylic acid; and with (3) an alkyl ester of a  $C_{2-10}$  olefinically unsaturated phosphonic acid, wherein the molecular ratios of said monomers is 11-300 moles of ethylene to 10 moles of the  $C_{8-20}$  alkyl ester of a  $C_{3-5}$  unsaturated carboxylic acid to 1-15 moles of the alkyl ester of a  $C_{2-10}$  olefinically unsaturated phosphonic acid, said terpolymer having a molecular weight of from 5,000 to 150,000.

2. The composition of claim 1 wherein the olefinically unsaturated phosphorus compound is diethyl isopropylidene phosphonate.

3. The composition of claim 1 wherein the alkyl ester of the unsaturated carboxylic acid is a mixture of lauryl and stearyl methacrylates and the alkyl ester of the olefinically unsaturated phosphonic acid is diethyl isopropylidene phosphonate.

4. The composition of claim 3 wherein the alkyl ester of the unsaturated carboxylic acid is diisooctyl itaconate.

\* \* \* \* \*